

C. L. WAGNER,  
FUEL AND PROCESS OF MAKING THE SAME,  
APPLICATION FILED APR. 7, 1919.

1,317,950.

Patented Oct. 7, 1919.

Fig. 1



Fig. 2



Witnesses  
A. E. Kinton  
Charles C. Collier

Inventor  
Charles L. Wagner  
By Dyer & Taylor  
Attorneys

# UNITED STATES PATENT OFFICE.

CHARLES L. WAGNER, OF NEW YORK, N. Y., ASSIGNOR TO S. STERNAU & COMPANY, INC.,  
OF BROOKLYN, NEW YORK, A CORPORATION OF NEW YORK.

## FUEL AND PROCESS OF MAKING THE SAME.

1,317,950.

Specification of Letters Patent.

Patented Oct. 7, 1919.

Application filed April 7, 1919. Serial No. 288,195.

*To all whom it may concern:*

Be it known that I, CHARLES L. WAGNER, a citizen of the United States, and a resident of the borough of Manhattan, city, 5 county, and State of New York, have invented a certain new and useful Fuel and Process of Making the Same, of which the following is a specification.

The invention relates to that class of fuel 10 known variously as solid alcohol, solidified alcohol or hard alcohol. Such a fuel is composed mainly of alcohol which is so mixed with other ingredients that the resulting product presents a solid mass which may 15 be handled, and which will retain its shape and form without being confined in a receptacle having the form in which the fuel is fashioned, and which will not melt under the heat of the flame which consumes it.

Such a fuel, as far as known, is composed 20 of a base of nitrated cotton or pyroxylin in which the alcohol is held. The proportion of pyroxylin to the alcohol must be relatively large in order that the alcohol will 25 be retained in the mass and be prevented from leaking out. Such fuels are objectionable, among other reasons, because of the fact that the relatively large amount of pyroxylin in burning will sputter and flash, 30 and sparks will be thrown off from the burning mass to a considerable distance. This is not only objectionable, but it also extremely dangerous.

The objects of the present invention are 35 to provide a solid fuel composed largely of alcohol, which will not melt, which will burn quietly but with an intense heat, which will deposit very little soot, which will not flash or sputter during combustion, which 40 will leave a very small amount of ash, which is non-explosive, which will be safe and cheap to manufacture, use and transport, and which will have no objectionable odor.

These and further objects will more fully 45 appear in the following specification and accompanying drawings considered together or separately.

One method of carrying out the process 50 and producing the solid fuel of the invention is illustrated in the accompanying drawings, in which like parts are designated by similar reference characters, and in which—

Figure 1 is a sectional view of a form of

apparatus for carrying out one step of the 55 process, and

Fig. 2 is a similar view of means for carrying out another step in the process.

In the drawings a tank 1 is illustrated. This tank may be of any desired construction and of any convenient size. In the bottom of the tank is located a pipe or coil 60 2 by means of which air or other fluid may be conveyed to the tank from a suitable source (not shown). Within the tank the 65 pipe or coil is perforated to permit of the escape of the air or other fluid.

Within the tank is placed a solution containing roughly 1 part ether and 4 parts alcohol 188 proof. The alcohol may be 70 pure or denatured, and for economic reasons denatured alcohol of United States Government formula No. 1, pyridin free, is employed. Into the ether-alcohol solution is placed carefully dehydrated cotton 75 in finely divided form, until the mixture assumes the consistency of honey. This solution is the preferred pyroxylin of the process.

To 188 proof denatured alcohol at a temperature of from 40° to 50° C. add a small quantity of ammonium nitrate. Of the ammonium nitrate alcohol solution take approximately three times the bulk of the pyroxylin, and stir a quantity of bagascello approximately equal in bulk to the pyroxylin into the alcohol ammonium nitrate solution. 80 85

The above mixture is now added to the pyroxylin in the tank 1 and air is forced 90 through the pipe 2 to aerate the mixture and remove part of the ether from the mass. The aeration will continue until the characteristic odor of the ether is barely noticeable.

Water in the form of a spray or jet is now 95 forced into the mixture, while the latter is being stirred slowly, until the mixture thickens. The thick mixture is put up in the form desired, and is ready for use.

Ammonium nitrate has a liquefying effect 100 on the solution when heated, thereby permitting dilution, without cracking of the pyroxylin beyond the point possible without the use of large quantities of ether, acetone, wood alcohol, or the higher alcohols. 105

If the fuel is to be dispensed in a can such as shown at 3 in Fig. 2 of the drawings the aerating and hydrating steps of the process

may be carried out in the can by admitting the water through a pipe 4. The water issuing under pressure from the perforations 5 of the pipe may be relied upon to agitate the mixture, or it may be agitated in any other manner as desired.

If the fuel is to be dispensed in the form of a cube, for example, all of the steps of the process, except the making of the alcohol ammonium nitrate bagascello mixture, may be carried out in the tank 1 and the water may be admitted through the pipe 2 after the mixture has been aerated.

It is important that the bagascello be added to the ammonium nitrate alcohol solution before the latter is mixed with the pyroxylin in order that it, the bagascello, may absorb as much of the alcohol ammonium nitrate solution as possible before the pyroxylin is mixed in.

The bagascello will absorb the alcohol ammonium nitrate solution freely and in addition, the solution will adhere to the surface of each particle of the bagascello. When the pyroxylin is added and the mixture is agitated the pyroxylin is distributed throughout the mass and the removal of the ether or the addition of water or both will cause the cotton to become partially precipitated and resume more or less its fibrous character and act as a binder for the saturated bagascello particles.

Such of the liquid content of the mixture as is not taken up by the bagascello will adhere to the partially precipitated cotton and there will be no free liquid in the mass.

Bagascello is readily combustible in the mixture, burns quietly and without flaring and sputtering and leaves less than 2% ash.

Ammonium nitrate when decomposed by the heat of combustion at the surface of the mass furnishes free oxygen, which causes complete combustion of the small particles of the partially precipitated cotton as they reach the surface and become dried. This will prevent the formation of a film of cotton on the surface of the mass and the consequent flaring as the relatively large amount of cotton becomes ignited. The burning surface of the fuel is always clean, and the heat of the flame is acting on fresh material at all times during burning. The oxygen released by the decomposition of the ammonium nitrate aids combustion and reduces sooting.

The base of the fuel is bagascello. Almost the entire liquid content is carried by the bagascello, and the relatively small amount of cotton present will, on its partial precipitation, form a net work throughout the mass and bind the liquid carrying particles together. The bagascello is not nitrated in the mixture, but its physical characteristics remain unchanged. It is simply a vehicle for carrying the liquid.

The bagascello used is the pith cell of the sugar cane as distinguished from the fibro vascular bundle cells. The pith elements are non-fibrous in structure, and are, in effect, bubbles of cellular material, filled with air. The alcohol-ammonium solution penetrates the walls of the bubbles by osmosis and displaces the air. Some of the solution adheres to the surface of the bagascello particles by adhesion. Bagascello will burn readily in the mixture before it becomes dry. In this respect it differs from cotton which must become dry before it will ignite.

The nitro-cellulose component of the fuel of the present invention is small and, because of the free oxygen at the burning surface of the mixture, each minute particle of it as it reaches the surface is ignited and the flare produced is so small as to be negligible and unnoticeable.

When the fuel is to be made in cube form and burned in a container which is not filled by the cube, a higher percentage of nitro-cellulose is desirable, because of the fact that the cubes must withstand more or less rough handling, and the liquid bearing particles should be more firmly bound together. When for use as just above described a 2% nitro-cellulose pyroxylin is desirable.

Instead of marketing the fuel in cans in which it is to be burned, or in air tight containers holding a number of bare cubes intended to be removed from the container and burned separately, the fuel may be put up in gelatin capsules of any desired size or shape. The capsules will prevent losses by evaporation and the fuel carrying capsules may be sold loose or in paper or cardboard cartons. When so packed the fuel may contain the low nitrated pyroxylin if desired. The fuel may be cut to fit the capsules or it may be made in the capsules.

To prevent sooty wood alcohol may be employed in the mixture. When wood alcohol is used it should not exceed 25% of the complete mass. A 10% wood alcohol content, is however preferable. The wood alcohol may form a part of the ammonium nitrate denatured alcohol solution by substituting the wood alcohol for an equal volume of denatured alcohol.

The wood alcohol may be added as the final step in the mixing, in which case a correspondingly smaller amount of denatured alcohol will be used in making the ammonium nitrate denatured alcohol solution.

While bagascello of sugar cane is, because of its cheapness and abundance, the preferred base material, it is to be understood that the pith of other plants such as corn, sorghum, elder, etc., may be employed.

The process carried out with the various materials in the following proportions gives good results:

In 5 grams of ether, and 20 grams of de-

natured alcohol 188 proof, is dissolved .9 gram of dehydrated cotton (preferably a mono-nitrate). This forms the pyroxylin.

A solution of from 1 to 5 grams of ammonium nitrate, and 75 grams of denatured alcohol 188 proof (pyrardin free), is made and heated to about 50° C., and to this mixture 21 grams, more or less, of bagascello is added, and the mixture is immediately 10 added to the pyroxylin. The mixture is then aerated to remove part of the ether, and while still limpid, approximately 88 grams of it are poured into a can such as that shown in Fig. 2. About 12 grams of water 15 in finely divided form is forced into the mass in the can causing an immediate solidification of the mass.

The aerating step of the process may be dispensed with and the water relied upon 20 to solidify the mixture.

A very satisfactory solid fuel may be made by soaking bagascello in alcohol (grain or wood) and when the bagascello has absorbed as much of the liquid as possible, the mass is placed in a can or other receptacle and is ready for use, or the can 25 may be filled or partly filled with bagascello and the alcohol poured therein until the limit of absorption is reached.

30 Instead of using bagascello as the base of the mixture any non-fibrous material which will absorb the liquid employed, and which will burn in the mixture may be used.

The addition of water in the process may 35 be dispensed with if desired. The removal of the ether by the air blast may be carried to such an extent as to partially precipitate the nitrated cotton, which is not soluble in grain alcohol. As the ether is removed the 40 percentage of the water content of the alcohol will be raised and this will materially assist in the partial precipitation of the nitro cellulose.

When making the ammonium nitrate alcohol 45 solution the former may be added in quantity sufficient to prevent cracking or precipitation of the mixture when rapidly added to the pyroxylin mixture while stirring. The ammonium nitrate may be as low 50 as 1% of the alcohol and should not be more than 5%.

In addition to the ammonium nitrate, any other material having the property of liberating free oxygen during combustion, and 55 being itself reduced may be employed. The use of such substances will assist combustion and reduce sootting. Examples of such materials are manganese, dioxid, and lead peroxid.

60 Bagascello is the name given in the West Indies to the interior, cellular, non-fibrous pith cells of bagasse or megass, as distinguished from the woody, fibrous portion of the sugar cane. It may be separated from 65 the hard, woody, fibrous outer-rind of the

cane by screening as is common in preparing the sifted bagasse or megass powder for the manufacture of molascuit, a stock food. The material may be further sifted by air flotation whereby the smallest and lightest 70 cellular, non-fibrous particles are recovered.

In accordance with the provisions of the patent statutes, the principle of the invention has been described together with what is now considered to be the best embodiment 75 thereof; but it is to be understood that the apparatus and process shown and described are merely illustrative, and that the invention may be carried out in other ways.

Having now described the invention what 80 is claimed and desired to be secured by Letters Patent is—

1. The process of making a solid fuel, which comprises adding alcohol to a cellular non-fibrous material. 85

2. The process of making a solid fuel, which comprises adding pyroxylin and alcohol to a cellular, non-fibrous material.

3. The process of making a solid fuel, which comprises adding pyroxylin, water 90 and alcohol to a cellular, non-fibrous material.

4. The process of making solid fuel, which comprises adding alcohol to a cellular, non-fibrous cellulose. 95

5. The process of making solid fuel, which comprises adding pyroxylin and alcohol to a non-fibrous cellulose.

6. The process of making solid fuel, which comprises adding pyroxylin, water and alcohol to a non-fibrous cellulose. 100

7. The process of making a solid fuel, which comprises adding alcohol to bagascello.

8. The process of making a solid fuel, 105 which comprises adding pyroxylin and alcohol to bagascello.

9. The process of making a solid fuel, which comprises adding pyroxylin, water and alcohol to bagascello. 110

10. The process of making a solid fuel, which comprises adding pyroxylin and alcohol to bagascello, and removing a portion at least of an ingredient of the pyroxylin.

11. The process of making a solid fuel, 115 which comprises adding pyroxylin and alcohol to bagascello, removing a portion at least of an ingredient of the pyroxylin, and adding water to the mass.

12. The process of making a solid fuel, 120 which comprises adding pyroxylin, alcohol and ammonium nitrate to a non-fibrous material.

13. The process of making a solid fuel, which comprises adding pyroxylin, alcohol, 125 ammonium nitrate and water to a non-fibrous material.

14. The process of making a solid fuel, which comprises adding pyroxylin, alcohol and ammonium nitrate to a non-fibrous ma- 130

4  
terial, and removing a portion at least of one ingredient of the pyroxylin.

15. The process of making a solid fuel, which comprises adding pyroxylin, alcohol and ammonium nitrate to a non-fibrous material, removing a portion at least of one ingredient of the pyroxylin, and adding water to the mixture.

16. The process of making a solid fuel, which comprises adding pyroxylin, alcohol, and ammonium nitrate to a non-fibrous cellulose.

17. The process of making a solid fuel, which comprises adding pyroxylin, alcohol, ammonium nitrate and water to a non-fibrous cellulose.

18. The process of making a solid fuel, which comprises adding pyroxylin, alcohol and ammonium nitrate to a non-fibrous cellulose, and removing a portion at least of one ingredient of the pyroxylin.

19. The process of making a solid fuel, which comprises adding pyroxylin, alcohol and ammonium nitrate to a non-fibrous cellulose, removing a portion at least of one ingredient of the pyroxylin, and adding water to the mixture.

20. The process of making a solid fuel, which comprises adding pyroxylin, alcohol and ammonium nitrate to a bagascello.

21. The process of making a solid fuel, which comprises adding pyroxylin, alcohol, ammonium nitrate and water to a bagascello.

22. The process of making a solid fuel, which comprises adding pyroxylin, alcohol and ammonium nitrate to a bagascello, and removing a portion at least of one ingredient of the pyroxylin.

23. The process of making a solid fuel, which comprises adding pyroxylin, alcohol and ammonium nitrate to a bagascello, removing a portion at least of one ingredient of the pyroxylin, and adding water to the mixture.

24. A process of making a solid fuel, which comprises dissolving nitrated cotton in ether and alcohol, mixing alcohol, ammonium nitrate and bagascello, adding the mixture to the solution, and removing a portion at least of the ether.

25. A process of making a solid fuel, which comprises dissolving nitrated cotton in ether and alcohol, mixing alcohol, ammonium nitrate and bagascello, adding the mixture to the solution, removing a portion at least of the ether, and adding water to the mixture.

26. The process of making a solid fuel,

which comprises dissolving a fibrous nitrated cellulose in ether and denatured alcohol, mixing bagascello in ammonium nitrate and denatured alcohol, adding the mixture to the solution, forcing air through the mass, and forcing water in finely divided condition into the mass.

27. The process of making a solid fuel, which comprises making a less than one per cent solution of mono-nitrate of cotton in approximately 5 parts ether and 20 parts denatured alcohol of high proof, dissolving approximately 5 parts ammonium nitrate in approximately 75 parts denatured alcohol of high proof, mixing approximately 2 $\frac{1}{2}$  parts of bagascello to the last named solution at a temperature of about 50° C., aerating the mixture to remove a portion at least of the ether, and adding approximately 12 parts of water to the mass.

28. A solid fuel, comprising a cellular, non-fibrous material and alcohol.

29. A solid fuel, comprising a cellular, non-fibrous cellulose and alcohol.

30. A solid fuel, comprising bagascello and alcohol.

31. A solid fuel, comprising bagascello, ammonium nitrate and alcohol.

32. A solid fuel, comprising bagascello, pyroxylin, ammonium nitrate, alcohol and water.

33. A solid fuel, consisting of a base comprising bagascello impregnated with alcohol, and a binder of partially precipitated pyroxylin.

34. A solid fuel, consisting of a base comprising bagascello impregnated with ammonium nitrate and alcohol, and a binder of partially precipitated pyroxylin.

35. A solid fuel, consisting of a base comprising bagascello impregnated with ammonium nitrate, water and alcohol, and a binder of partially precipitated pyroxylin.

36. A solid fuel, comprising bagascello, nitrocellulose, ether, alcohol and ammonium nitrate.

37. A solid fuel, comprising bagascello, nitrocellulose, ether, alcohol, water and ammonium nitrate.

38. A solid fuel, comprising a cellular non-fibrous material, nitro-cellulose, ether, alcohol, water and ammonium nitrate.

This specification signed and witnessed this second day of April, 1919.

CHARLES L. WAGNER.

Witnesses:

J. F. COLEMAN,  
A. E. RENTON.